

## UNITED STATES PATENT OFFICE

2,084,516

## PROCESS OF MANUFACTURING TEXTILE ARTICLES

Julien Van Puymbroeck, Brussels, Belgium

No Drawing. Application March 9, 1935, Serial No. 10,150

5 Claims. (Cl. 19—66)

In textile articles, such as yarn, fabrics, hosiery and the like, solidity is secured by producing during the spinning operation an entanglement of the hooks or scales of the textile fibres, when use is made of fibres having such hooks, for instance certain qualities of wool, or by agglomerating the fibres of the yarn or yarns from which the fabrics or articles of hosiery are formed, by felting, such agglomeration being produced also by the fulling mill, or by both means in combination.

It is known furthermore, that during the spinning operation, it is generally needed to oil the materials to be spun, and this as well in the combed spinning industry as in the carded spinning industry. The oiling product generally used is olein.

It is thus only possible, in a general manner, to produce a knitted article, a fabric or a yarn of resistant quality by means of textile fibres of animal origin when use is made of fibres having hooks allowing the entanglement of said fibres with each other, or of fibres having a felting capacity which they keep during the spinning operations and namely after the oiling, and which allows to agglomerate such fibres by felting.

Certain fibres of animal origin do not have such natural felting capacity, and such are particularly the hairs of domestic or wild rabbits and the hairs of hares, or such fibres have only this felting capacity to a degree insufficient to be agglomerated in a sufficiently resistant manner by felting; such fibres however may acquire artificially a felting capacity or at least increase considerably this capacity, namely by a chemical operation known in the art under the notion "secreting operation", and which modifies the appearance of the fibre when viewed in the microscope.

The secreting gives to the fibres a felting capacity which allows them to solidly agglomerate in a mass when they are conveniently treated.

It is therefore that in the hat-making industry a considerable use is made of secreted rabbit and hare's hair for the manufacturing of hats of high quality.

In spinning, however, it has been stated that the secreted animal fibres and more particularly the hair of domestic and wild rabbits and of hares lose their felting capacity when they are being oiled by means of olein or the other oiling substances commonly used in the spinning industry.

In the description hereafter, the expression "secreted fibres" will be used as a generic designation for all animal fibres and more particularly for hair of domestic and wild rabbits or of hares which do not possess a felting capacity or only possess naturally a felting capacity insufficient for allowing them to agglomerate in a solid mass, and which, by any chemical process, have artificially acquired a sufficient felting capacity, which however disappears when the fibre is coated with olein or any other substances containing a fatty material. In the same direction, the expression "felting capacity" will be used for designating the capacity of agglomerating in a resistant and solid mass by felting. The term "yarn" will be used to designate the twisted yarns presenting a certain degree of twist and manufactured by spinning.

It has already been proposed to mix a quantity of hair and namely of certain qualities of Angora rabbit hair with wool for manufacturing yarn and afterwards fabrics having a silky feel and a nice appearance in conformity with the fashion. But in the articles of this kind, the hair is only enclosed within the mass of wool and is readily removed by a simple stretching action. This effect may be explained by the fact that said hairs have no hooks or scales and having been oiled with olein or with a similar fatty or oily substance or the like, they do not possess any felting capacity or only possess a deficient degree thereof, so that they cannot become agglomerated by felting or entangled with the hooks or scales of the wool fibres.

The invention consists in a method of manufacturing a new article formed by a fabric or a knitted article or manufactured yarn, either in carded or in combed material, and formed either by means of secreted fibres or by means of a mixture of secreted fibres and other fibres, and in which, contrarily to what has been the case for all fabrics and articles of hosiery actually manufactured, the secreted fibres are agglomerated by felting.

This method of manufacturing is mainly characterized by the fact that the materials to be spun, formed by secreted fibres or containing secreted fibres in mixture with other fibres, are oiled no longer with olein or by means of other known oiling substances, but by means of a substance containing slimy or mucilaginous products.

According to the invention, the materials to be spun may be oiled by means of a product containing a decoction of leaves, branches or roots of malvaceous plants and for instance a decoction of mallow roots.

- According to the invention, the oiling may be generally performed by means of a decoction of a mixture of malvaceous plants and for instance of mallow roots and plants of the order of the compositae and namely of tussilage also named colt's foot.
- Such decoction may be made as well with the roots as with the leaves, flowers, seeds or any other part of the plants.
- 10 According to another object of the invention, the fabric or hosiery article manufactured by means of this yarn, or the yarn itself, may be fulled with an acid bath in order to secure an agglomeration of the fibres by felting.
- 15 Various compositions of baths may be convenient. By way of example, use may be made of a bath containing a solution of sulphuric acid at 1 to 2° Bé., or a solution of lactic acid of 1 to 3° Bé.
- 20 The fabrics, hosiery articles and other finished articles containing wholly or partly twisted yarn comprising secreted hair having a felting texture according to the invention and treated according to the invention, will present numerous ad-
- 25 vantages over woolen fabrics. As such may be cited namely, that they are warmer and lighter in wearing, they are waterproof or may be water-proofed, present a nice appearance and feel, they are extremely resistant and present electric prop-
- 30 erties favourable for curing certain diseases, such as rheumatism.
- I claim:
1. A process of spinning a material containing secreted fibres consisting in oiling the material 35 by means of a product containing a decoction of
- malvaceous plants and spinning such oiled mass of material according to convenient methods.
2. A process of spinning a material containing secreted fibres consisting in oiling the material by means of a product containing a decoction of 5 mallow roots and plants of the order of the compositae, such as tussilage (colt's foot), and spinning such oiled mass of material according to convenient methods.
3. A process of spinning a material containing secreted fibres consisting in oiling the material 10 by means of a product containing a decoction of a mixture of malvaceous plants, such as mallow roots, and of plants of the order of the compositae, such as tussilage (colt's foot), and spinning such oiled mass of material according to 15 convenient methods.
4. A process of manufacturing a textile article containing yarn comprising secreted fibres, consisting in oiling the mass of material to be spun by means of a substance containing a mucilag- 20 inous product; spinning this material according to a convenient method, producing by means of such yarn a textile article such as a fabric, hosiery and the like, and felting the thus produced textile article in an acid bath. 25
5. A process of manufacturing a textile article containing yarn comprising secreted fibres, consisting in oiling the mass of material to be spun by means of a substance containing a decoction of malvaceous plants such as mallow roots, spin- 30 ning this material, producing by means of the yarn obtained a textile article such as a fabric, hosiery and the like, and fulling such article in an acid bath.

JULIEN VAN PUYMBROECK. 35